

[54] PROCESS FOR PRODUCING  
1,5-DIACETYL-3,7-DINITRO-1,3,5,7-  
TETRAAZACYCLOOCTANE[75] Inventors: Michael D. Coburn, Los Alamos;  
Theodore M. Benziger, Santa Fe,  
both of N. Mex.[73] Assignee: The United States of America as  
represented by the United States  
Energy Research and Development  
Administration, Washington, D.C.

[22] Filed: Dec. 5, 1974

[21] Appl. No.: 529,988

[52] U.S. Cl. .... 260/239 BC

[51] Int. Cl.<sup>2</sup> .... C07D 257/02

[58] Field of Search .... 260/239 BC, 239 HM

## [56] References Cited

## OTHER PUBLICATIONS

Yoshida et al., J. of Heterocyclic Chem., Vol. 10, pp.  
727-730 (1973).Topchieu Nitration of Hydrocarbons and Other Or-  
ganic Compounds, p. 62 permogen 1962.

Primary Examiner—Donald G. Daus

Assistant Examiner—W. B. Springer

Attorney, Agent, or Firm—Dean E. Carlson; Edward  
C. Walterscheid

## [57] ABSTRACT

Diacetyl pentamethylene tetramine in solution in acetic acid is converted to 1,5-diacetyl-3,7-dinitro-1,3,5,7-tetraazacyclooctane by nitrolysis in a mixture of nitric and sulfuric acid. The amount of nitric acid required for this purpose may be reduced to near-stoichiometric levels and a resultant hazardous exothermic reaction avoided by the addition of urea to the acetic acid solution of diacetyl pentamethylenetetramine before nitrolysis occurs.

4 Claims, 2 Drawing Figures



Fig. 1



Fig. 2

**PROCESS FOR PRODUCING  
1,5-DIACETYL-3,7-DINITRO-1,3,5,7-TETRAAZACYCLOOCTANE**

**BACKGROUND OF THE INVENTION**

The invention described herein was made in the course of, or under, a contract with the U.S. ATOMIC ENERGY COMMISSION. It relates to high explosives and, more particularly, to an improved method for preparing 1,5-diacetyl-3,7-dinitro-1,3,5,7-tetraazacyclooctane; an intermediate in a preferred synthesis of the high explosive cyclotetramethylenetrinitramine.

Cyclotetramethylenetrinitramine (HMX) is a powerful high explosive possessing significant advantages in both explosive performance and thermal stability over other explosives such as the widely used cyclotrimethylenetrinitramine (RDX). Because of its high cost (~3 to 4 times that of RDX) it typically finds use only in specialized ordnance such as shaped charges, where the explosive performance must be maximized. Presently, HMX is manufactured by a modified version of the Bachmann RDX process.

Another process has recently been developed, however, which results in substantially greater yields of HMX than can be obtained by the modified Bachmann RDX process, even though it uses essentially the same raw materials. A mixture of hexamethylenetetramine (hexamine), acetic anhydride, and ammonium acetate is reacted to form diacetyl pentamethylenetetramine (DAPT) produced as a solution in acetic acid. This crude solution is then added to a mixture of nitric and sulfuric acids, where it is converted to 1,5-diacetyl-3,7-dinitro-1,3,5,7-tetraazacyclooctane (DADN). This product is recovered in high yield (94%, based on hexamine). In a subsequent nitrolysis step the DADN is converted to HMX.

For the nitrolysis of DAPT to DADN in accordance with this process to be economically feasible, it is desirable that a good yield of high-purity DADN be obtained by using a near-stoichiometric amount of nitric acid. In addition, a short reaction time is advantageous if a continuous rather than a batch process is to be used. The art discloses that good yields of high-purity DADN can be obtained but only through use of a ten-fold excess of nitric acid and a reaction time of 100 minutes. A significant problem, however, is that if the nitric acid concentration is reduced to a near-stoichiometric level, a violent abrupt exotherm occurs toward the end of the reaction. Such an exotherm constitutes an intolerable hazard in any large-scale process.

**SUMMARY OF THE INVENTION**

In accordance with the present invention, the violent exotherm which results from the nitrolysis of DAPT to DADN with near-stoichiometric concentrations of nitric acid may be completely eliminated by the addition of urea to the crude solution of DAPT in acetic acid prior to the nitrolysis. The urea addition not only avoids the production of the exotherm but also allows the temperature of the nitrolysis step to be increased and the nitrolysis to be completed in a substantially shorter time than is taught in the prior art.

**BRIEF DESCRIPTION OF THE DRAWINGS**

FIG. 1 shows a representative example of the exotherm which occurs during the nitrolysis of DAPT in

acetic acid solution with a near-stoichiometric amount of nitric acid in the absence of urea.

FIG. 2 is a comparison of the yield of DADN produced during the nitrolysis of a standard DAPT feed solution at 30°C with and without the presence of urea.

**Nitrolysis of DAPT to DADN**

The literature discloses that DADN may be prepared by the nitrolysis of DAPT to DADN using a mixture of nitric and sulfuric acids. See, e.g., Yoshida et al., "Synthesis of 1,3,5,7-tetraazacyclooctane Derivatives," *J. Heterocyclic Chem.* 10, 725 (1973). It is also known that hexamine, acetic anhydride, and ammonium acetate may be advantageously reacted to form DAPT in acetic acid solution. By way of example only, 0.1 mole of DAPT in solution in acetic acid may readily be prepared by blending 0.1 mole hexamine, 0.081 mole ammonium acetate, and 0.39 mole H<sub>2</sub>O into a slurry in a 50-ml flask held at 5° to 10°C and adding 0.3 mole acetic anhydride to the stirred slurry over a 60 min. period while holding the reaction temperature at 5° to 10°C.

It is desirable to be able to perform the nitrolysis of the DAPT using the acetic acid solution rather than pure DAPT. A preferred procedure for doing this in the prior art is indicated by the following example. A mixed acid is prepared from 1.0 mole of 99% HNO<sub>3</sub> and 2.26 moles of 96% H<sub>2</sub>SO<sub>4</sub>. The crude DAPT in solution in acetic acid prepared in accordance with the foregoing example is added dropwise to the acid mixture over a period of 50 min. with the reaction temperature held at 18° to 20°C and the resultant reaction mixture aged for 20 min. at 20°C. The reaction mixture is then quenched with 1,000 g of ice and the DADN precipitated with the addition of 1,500 ml of water. The filtered product consists of 0.095 mole DADN which is a 95% yield. The reaction is:



It is to be noted that in this example of the preparation of DADN, a substantial excess of HNO<sub>3</sub> has been used, the reaction temperature has been kept at 20°C or less, and the reaction time is of the order of 70 minutes. When the concentration of HNO<sub>3</sub> is reduced to near-stoichiometric levels, the exotherm shown in FIG. 1 results. Although the nitrolysis of dry DAPT can be accomplished without a delayed exotherm, the yield is lower than when water and acetic acid are present.

**DESCRIPTION OF THE PREFERRED EMBODIMENT**

The amount of HNO<sub>3</sub> required for the nitrolysis of DAPT in solution in acetic acid to DADN may be reduced to near-stoichiometric concentrations and the reaction temperature and reaction rates increased without adversely affecting the yield of DADN through the addition of urea to the crude DAPT solution before nitrolysis is commenced. The effect of the addition of urea when the HNO<sub>3</sub> concentration is reduced to a near-stoichiometric level and the reaction temperature increased to 30°C is shown by comparing the data of FIG. 2 and Tables I through III. These data are obtained using a DAPT feed solution prepared by adding 0.25 mole acetic anhydride to a slurry of 0.10 mole hexamine and 0.082 mole ammonium acetate in 0.139 mole (2.5 ml) water. The nitrolysis medium is made up of 0.33 mole 90% HNO<sub>3</sub> and 2.25 mole 98% H<sub>2</sub>SO<sub>4</sub>. The DAPT feed solution is added to the nitrolysis medium over a 6-min. period with the temperature during

the addition controlled between 30° and 35°C with ice-water cooling.

TABLE I

| Time (min) | DADN Yield (moles) | Purity (%) | CH <sub>2</sub> O (moles) | Spent Acids HNO <sub>3</sub> (moles) | HNO <sub>2</sub> (moles) |
|------------|--------------------|------------|---------------------------|--------------------------------------|--------------------------|
| 10         | 0.058              | 97         | 0.30                      | 0.028                                | 0.0001                   |
| 15         | 0.092              | 90         | 0.18                      | 0.024                                | 0.006                    |
| 30         | 0.087              | 98         | 0.08                      | 0                                    | 0.030                    |

TABLE II

| Time (min) | DADN Yield (moles) | Purity (%) | CH <sub>2</sub> O (moles) | Spent Acids HNO <sub>3</sub> (moles) | HNO <sub>2</sub> (moles) |
|------------|--------------------|------------|---------------------------|--------------------------------------|--------------------------|
| 10         | 0.081              | 100        | 0.24                      | 0.028                                | 0                        |
| 20         | 0.091              | 100        | 0.20                      | 0.027                                | 0.001                    |
| 30         | 0.093              | 100        | 0.20                      | 0.026                                | 0.004                    |
| 40         | 0.093              | 100        | 0.19                      | 0.022                                | 0.008                    |
| 50         | 0.093              | 100        | 0.17                      | 0.017                                | 0.017                    |
| 60         | 0.091              | 100        | 0.17                      | 0.009                                | 0.026                    |

TABLE III

| Time (min) | DADN Yield (moles) | Purity (%) | CH <sub>2</sub> O (moles) | Spent Acids HNO <sub>3</sub> (moles) | HNO <sub>2</sub> (moles) |
|------------|--------------------|------------|---------------------------|--------------------------------------|--------------------------|
| 10         | 0.084              | 100        | 0.21                      | 0.034                                | 0                        |
| 20         | 0.095              | 100        | 0.19                      | 0.028                                | 0.0001                   |
| 30         | 0.093              | 100        | 0.19                      | 0.030                                | 0.0003                   |
| 40         | 0.094              | 100        | 0.18                      | 0.030                                | 0.0003                   |
| 50         | 0.093              | 100        | 0.18                      | 0.027                                | 0.0006                   |
| 60         | 0.092              | 100        | 0.18                      | 0.031                                | 0.0009                   |
| 115        | 0.092              | 100        | 0.17                      | 0.026                                | 0.0034                   |

As is shown by FIG. 2 and Table I, increasing the reaction temperature to 30°C without adding urea to the DAPT feed solution increases the rate of nitrolysis but at the expense of a significant decrease in the DADN yield. Without the presence of urea, a 90°C exotherm also occurs at 19 minutes. The addition of either 0.05 mole (FIG. 2 and Table II) or 0.1 mole (Table III) of urea effectively prevents the exotherm

and permits rapid nitrolysis at 30°C. A mild, easily controlled exotherm occurs when the urea is reduced to 0.02 mole. At 40°C, using 0.05 mole of urea, no exotherm is observed and the reaction is complete within 10 min. after the addition of the DAPT solution is initiated. No reduction in yield occurs under the latter conditions.

The manner in which the urea acts to prevent the exotherm while allowing the higher DADN yield at the faster reaction rate permitted by the higher reaction temperatures is not completely understood. It appears, however, that the exotherm is produced by the abrupt oxidation of a substantial amount of the formaldehyde generated as a byproduct during the nitrolysis. As is indicated in Tables II and III, the addition of urea prevents the destruction of formaldehyde and retards the reduction of nitric acid. When 0.1 mole of urea (Table III) is added to the DAPT feed solution the conversion of nitric to nitrous acid is completely inhibited, while with the addition of 0.05 mole of urea (Table II) this conversion is essentially complete in 60 min. The mode of action of urea in preventing the destruction of formaldehyde does not appear to be related to its ability to destroy nitrous acid, but it may be protecting the formaldehyde by forming an adduct, such as dimethylol urea.

What we claim is:

1. In a method for preparing 1,5-diacetyl-3,7-dinitro-1,3,5,7-tetraazacyclooctane by the nitrolysis in mixed HNO<sub>3</sub>—H<sub>2</sub>SO<sub>4</sub> of diacetyl pentamethylenetetramine in solution in acetic acid, the improvement comprising the addition of urea to said acetic acid solution of diacetyl pentamethylenetetramine before said nitrolysis.
2. The method of claim 1 wherein the concentration of said HNO<sub>3</sub> is slightly in excess of the stoichiometric amount required for said nitrolysis.
3. The method of claim 2 wherein said nitrolysis occurs at about 40°C.
4. The method of claim 2 wherein said urea is added in an amount sufficient to react completely with the formaldehyde formed during said nitrolysis.

\* \* \* \* \*